

# UNITED STATES PATENT OFFICE.

OTTO NEUBERGER, OF FRANKFORT-ON-THE-MAIN, GERMANY.

## PROCESS OF OBTAINING PRINTS ON FABRICS.

1,135,043.

Specification of Letters Patent. Patented Apr. 13, 1915.

No Drawing.

Application filed February 27, 1914. Serial No. 821,557.

To all whom it may concern:

Be it known that I, OTTO NEUBERGER, manufacturer, a citizen of the Empire of Germany, residing at Frankfort-on-the-Main, Germany, have invented certain new and useful Improvements in the Process of Obtaining Prints on Fabrics, of which the following is a specification.

My present invention relates to the printing of fabrics by means of reduction-dye-stuffs. I have found that reduction-dye-stuffs, such as vat- or sulfur-dye-stuffs, which are remarkable for their fastness, can be fixed on fabrics with the aid of the lithographic or book-printing process by applying the dyestuff, after being very finely ground together with a varnish or an oil, upon the fabric previously prepared with an alkali and a reducing-agent, and fixing the thus applied dyestuff by subsequent steaming.

The prints obtained by the above-mentioned process are of excellent fastness to washing and rubbing, because, in consequence of the reduction effected by the steaming, the color is thoroughly fixed on the fiber. This result is an unexpected one inasmuch as it could not be foreseen that the presence of a varnish produces no detrimental effect upon the reduction and fixing of the dyestuff and the purity of the prints obtainable thereby. The process may be modified by first printing the color and subsequently applying the alkali and the reducing agent.

Furthermore I have found that the reducing substance serving as an agent for the fixing of the color may also, with advantage, be added to the lithographic or book-printing-color containing varnish. In this case no reducing agent or only a small quantity of it need be used for the preparation of the fabric, whereby a great saving is effected. This also renders it possible to conform in every case the quantity of the reducing agent to be used exactly to the quantity of the dyestuff, whereby more even prints are obtained. For this process the insoluble, stable hydrosulfite compounds are particularly suitable. The reduction-dye-stuffs may also be used in the form of their leuco compounds for the preparation of the printing colors. For the impregnation of

the fabric there may, for instance, be used a solution of the following composition: 55 30 grams of wheat starch; 895 grams of water heated to boiling, and added lukewarm; 50 grams of calcined sodium carbonate; 25 grams of hydrosulfite NF concentrated. 60

The following examples illustrate my invention:

Example I: 150 grams of helindone violet R powder (4,4-dimethyl-5,5-dichloro-7,7-dimethoxythioindigo) are finely ground in 65 the usual manner together with 100 grams of printers' varnish and printed on the fabric previously prepared and calendered. After drying, the goods are steamed for 5 minutes or longer above 100° C., preferably with steam free from air, and then 70 well washed and soaped at the boil for completely developing the shade, whereupon they are again washed and dried. Instead of previously preparing the fabric, the impregnation of the unprepared fabric may 75 be effected with the above-mentioned impregnating-liquid after the color has been applied.

Example II: The fabric may be prepared with a solution of the following composition: 80 30 grams of wheat starch are boiled with 920-987 grams of water and there are then added lukewarm 50-100 grams of calcined sodium carbonate. The 85 fabric to be printed is impregnated with this solution, then dried and calendered.

The printing-process is carried out as follows: 100 grams of helindone red 3B powder (5,5-dichloro-7,7-dimethylthioindigo) are 90 finely ground together with 300 grams of zinc-formaldehyde-sulfoxylate and 200 grams of varnish and printed on the fabric prepared with alkalis as above indicated. After well drying, the fabric is steamed for 95 5 minutes or longer above 100° C., well washed and soaped at the boil for completely developing the shade, and finally again washed and dried.

Example III: The procedure is the same 100 as indicated in Example II except that the composition of the printing-color is to be as follows: 100 grams of helidone red 3B in form of its leuco compound, 150 grams of zinc formaldehydesulfoxylate, 350 grams 105 of varnish.

It may be remarked that in all of the three examples the quantity of the alkali and the reducing agents may be varied within wide limits, accordingly as required.

5 Having now described my invention what I claim is:

1. The process of obtaining designs on fabrics, which consists in applying on the fabric reduction dyestuffs finely ground with varnish or an oil by means of the lithographic printing process and developing the prints thus obtained by steaming in presence of an alkali and reducing agents.
- 10 2. The process of obtaining designs on fabrics, which consists in applying on the fabric reduction dyestuffs in the form of leuco compounds finely ground with varnish or an oil by means of the lithographic printing process, and developing the prints thus obtained by steaming in presence of an alkali and reducing agents.
- 15 3. The process of obtaining designs on fabrics, which consists in first impregnating the fabric with a solution of an alkali and reducing agents, then applying reduction dyestuffs finely ground with varnish or an oil by means of the lithographic printing process, and developing the prints thus ob-

tained by steaming in presence of an alkali and reducing agents.

4. The process of obtaining designs on fabrics, which consists in first impregnating the fabric with an alkali, then applying reduction dyestuffs mixed with a reducing agent and finely ground with varnish or an oil, by means of the lithographic printing process, and developing the prints thus obtained by steaming in presence of an alkali and reducing agents.

5. The process of obtaining designs on fabrics, which consists in first impregnating the fabric with an alkali and part of the reducing agents, then applying reduction dyestuffs mixed with the other part of the reducing agents and finely ground with varnish or an oil, by means of the lithographic printing process, and developing the prints thus obtained by steaming in presence of an alkali and reducing agents.

In testimony whereof I affix my signature in presence of two witnesses.

OTTO NEUBERGER.

Witnesses:

JEAN GRUND,  
CARL GRUND.